# EUROPEAN PATENT SPECIFICATION

(11) **EP 1 719 634 B1**
(45) Date of publication and mention of the grant of the patent: **18.03.2009**
(21) Application number: 06113009.2
(22) Date of filing: 24.04.2006
(51) Int. Cl.: B41M 3/00, B41M 3/14

(54) **Authenticable coated paper material, in particular for labelling and packaging, and manufacturing method thereof**
Gestrichenes Sicherheitspapier, insbesondere für Etiketten und Verpackungen, und Verfahren zu dessen Herstellung
Papier de sécurité couché, en particulier pour étiquettes et emballage, et procédé de fabrication

(30) Priority: 26.04.2005 IT MI20050744
(43) Date of publication of application: 08.11.2006
(73) Proprietor: GRUPPO CORDENONS S.p.A., 20145 Milano (IT)
(72) Inventor: Gilberti, Ferruccio, 20121, Milano (IT); Monacelli, Luca, 33170, Pordenone (IT)
(74) Representative: Jorio, Paolo

(56) References cited:
- WO-A-98/33654
- GB-A- 2 052 587
- US-A- 4 022 771
- US-A- 4 037 007
- US-A- 5 250 492
- US-A- 5 318 939
- US-A- 5 329 006

## Description

The present invention relates to an authenticable coated paper material, in particular for labelling and packaging, to the manufacturing method thereof, and to an authentication kit, in particular for labels and/or packages, using such paper material.

Various so-called security papers, i.e. papers provided with various artifices having the function of avoiding or highlighting possible illicit reproduction or forgery, are known; in particular, security papers are known whose composition incorporate substances sensitive to particular external treatments aimed, precisely, to reveal the presence of such substances.

This type of paper is not free from drawbacks, both during the manufacturing process (firstly because they require the inclusion of sensitive substances directly in the pulp during the paper manufacturing process, which requires particular precautions and care), and at the moment of use, because they generally require the use of relatively complex and costly authentication tools. Furthermore, the inclusion of sensitive substances in the paper composition compromises to a certain extent the final features of the product, above all in terms of printability, and indeed these papers are not generally suitable for high quality printing, typical of glossy coated paper. On the other hand, these papers cannot be coated, because coating would compromise the efficacy of the sensitisation treatment.

Other known security papers also present similar printing problems, because the security treatments, generally, indeed compromise printability.

Examples of the known authenticable papers are disclosed in the following documents: US-A-4 037 007, US-A-5 250 492, WO 98/33654, US-A-4 022 771.

Document GB-A-2 052 587 discloses an authenticable coated paper material comprising a paper support and a coating applied to said support, said coating comprising oxidised starch and a chromogen composition sensitive to application of an activating composition and adapted to generate a visible marking following the application of the activating composition.

It is an object of the present invention to provide a paper material which is free from the drawbacks of the prior art here described; in particular, it is an object of the invention to provide a paper material which is printable with high printing quality using traditional printing techniques and which is at the same time simply and efficaciously authenticable, being also relatively simple and cost-effective to manufacture.

The present invention therefore relates to an authenticable glossy coated paper material, in particular for labelling and packaging, comprising a paper support and a coating applied on at least one side of the support and printable with high printing quality, the material being characterised in that the coating is made of a polymeric coating composition comprising a polymerizable base mixed with kaolin, inert filters, casein and possible other additives and incorporating a chromogen composition sensitive to application of an external activating composition and adapted to generate a visible marking following the application of the external activating composition.

In particular, the chromogen composition is adapted to react with a reactant or solvent contained in the activating composition to release a colouring in the coating and generate the marking.

According to the invention, the chromogen composition includes at least one xanthene colourant, i.e. a colourant with oxygen-containing heterocyclic chromophores and/or at least one encapsulated colourant, in particular a pre-dispersed grease colourant.

In this way, the chromogen composition is sensitive to a chlorine-derivative based activating composition, in particular to an activating composition containing chloro-derivative inorganic acid salts, for example a hypochlorite solution, or organic chloro-derivatives, for example perchloroethylene, and/or to a solvent based activating composition, in particular a polar or apolar organic solvents based composition.

The invention also relates to an authentication kit, in particular for labels and/or packages, comprising the coated paper material described above and an authentication felt-tip pen adapted to release the activating composition to highlight the chromogen composition in the paper material coating.

In particular, the activating composition includes a reactant or solvent adapted to react with the chromogen composition to release a colouring in the coating.

The authentication felt-tip pen therefore contains a chloride derivate based activating composition, in particular an activating composition containing chloride derived inorganic acid salts, for example a hypochlorite solution, or organic chloro derivatives, for example perchloroethylene, and/or a polar or apolar organic solvent-based activating composition (according to the chromogen composition present in the coating).

The paper material described above is manufactured, according to a further aspect of the present invention, using the following method.

The paper support of essentially known type, for example a cellulosic base paper having a traditional composition and, preferably, a substance ranging between approximately 50 and 500 g/m², is first manufactured in a known way.

A polymeric coating composition is then prepared, comprising a polymerizable base (acrylic, polyurethane, polyolefinic, etc.) mixed with kaolin, inert fillers (e.g. carbonate in crystalline form), casein and possible other (known) additives.

The chromogen composition described above is added to the coating composition.

The coating composition incorporating the chromogen composition is therefore applied, in a quantity ranging between approximately 1 and approximately 50 g/m² and preferably between approximately 5 and approximately 20 g/m² (dry) on one side (or also on both sides) of the paper support, so as to form a coated glossy surface, which is printable with high printing quality and authenticable by applying the external activating composition.

The coating composition is applied by spreading with an air-blade or sliding-blade coating machine.

A heating step then follows to dry and polymerise the coating composition to form the coating. The heating step is performed in infrared and/or hot air oven, at temperatures from approximately 100°C to 180°C and permanence time in the oven of approximately 0,5 to 4 minutes.

The material after traditional finishing steps is used in particular to make labels (e.g. for wine, beverages and foodstuff in general) and/or boxes, packages and wrappings of various types.

The advantages of the present invention are clear from the foregoing description. The paper material according to the invention allows indeed to manufacture labels and/or packages with excellent graphic quality, and also allows rapid and secure authentication.

The paper material according to the invention is indeed perfectly printable with the usual printing techniques, in particular ink printing techniques, with high printing quality; at the same time, the paper material of the invention may be easily and rapidly authenticated to verify that it is an original material (and therefore applied to an original item). For verifying authenticity, it is sufficient to pass the authentication felt-tip pen on the coated surface of the paper material so as to make the chromogen composition, present in the coating, react with the external activating composition, released by the authentication felt-tip pen, and generate a visible marking.

Instead, if following the passage of the authentication pen no marking is detected, it means that the paper material is a fake, and not an original.

The manufacturing method is also simple and cost-effective, in particular because the chromogen composition is not directly incorporated in the paper support (i.e. incorporated in the paper material mass) but is added to the coating composition before it is spread on the paper support; the chromogen composition is therefore present in the coating and not in the mass of the paper support.

The invention is further described by way of example in the following non-limiting embodiments.

### EXAMPLES

Various series of paper supports having substance of 50, 90, 120, 150, 200, 250, 350, 500 g/m², and various coating compositions (mixtures of different polymeric materials, kaolin, fillers and casein in various ratios) were prepared using the method described above.

Xanthene colourants and/or encapsulated colourants, in particular pre-dispersed grease colourants, available on the market, were added to the coating compositions.

The resulting compositions were then applied to one or both sides of the paper supports in variable amounts, in particular 1, 5, 10, 15, 20, 35, 50 g/m², using the procedure described above.

The paper material obtained were printed using traditional techniques, with excellent graphic quality, and tested by passing an authentication felt-tip pen on the coated surfaces.

## Claims

1. An authenticable coated paper material for labelling and packaging, comprising a paper support and a glossy coating applied on at least one side of the support and printable with high printing quality; wherein
the coating is made of a polymeric coating composition comprising a polymerizable base mixed with kaolin, inert fillers, casein and possible other additives; and incorporating a chromogen composition sensitive to application of an external activating composition and adapted to generate a visible marking following the application of the external activating composition; the chromogen composition including at least one xanthene colourant and/or an encapsulated colourant.

2. A paper material according to claim 1, **characterised in that** the chromogen composition is adapted to react with a reactant or solvent contained in the activating composition so as to release a colouring in the coating and generate the marking.

3. A paper material according to one of the preceding claims, **characterised in that** the encapsulated colourant is a pre-dispersed grease colourant.

4. A paper material according to one of the preceding claims, **characterised in that** the chromogen composition is sensitive to a chlorine-derivative based activating composition.

5. A paper material according to one of the preceding claims, **characterised in that** the chromogen composition is sensitive to an activating composition containing chloro-derivative inorganic acid salts or organic chloro-derivatives.

6. A paper material according to one of the preceding claims, **characterised in that** the chromogen composition is sensitive to a solvent based activating composition, in particular a polar or apolar organic solvents based composition.

7. An authentication kit for labels and/or packaging, comprising a coated paper material according to one of the preceding claims and an authentication felt-tip pen, adapted to release said activating composition to highlight the chromogen composition in the coating.

8. An authentication kit according to claim 7, **characterised in that** the activating composition includes a reactant or solvent adapted to react with the chromogen composition to release a colouring in the coating.

9. An authentication kit according to claim 7 or 8, **characterised in that** the authentication felt-tip pen contains a chlorine-derivative based activating composition.

10. An authentication kit according to claim 9, **characterised in that** the activating composition contains chloro-derivative inorganic acid salts and/or organic chloro-derivatives.

11. An authentication kit according to one of the claims from 7 to 10, **characterised in that** the authentication felt-tip pen contains a solvent-based activating composition, in particular a polar or apolar organic solvents based composition.

12. A method for manufacturing an authenticable coated paper material for labelling and packaging, comprising the steps of: providing a paper support; preparing a polymeric coating composition comprising a polymerizable base mixed with kaolin, inert fillers, casein and possible other additives; adding to the coating composition a chromogen composition sensitive to the application of an external activating composition adapted to generate a visible marking following the application of the external activating composition and including a xanthene colourant and/or an encapsulated colourant; applying the coating composition incorporating the chromogen composition on one side of the support to form a glossy printable coating with high printing quality and authenticable by applying the external activating composition.

13. A method according to claim 12, **characterised in that** the chromogen composition is adapted to react with a reactant or solvent contained in the activating composition so as to release a colouring in the coating and generate said marking.

14. A method according to claims 12 or 13, **characterised in that** the chromogen composition is sensitive to a chlorine-derivative based activating composition and/or a solvent based activating composition, in particular a polar or apolar organic solvents based composition.

## Patentansprüche

1. Authentifizierbares beschichtetes Papiermaterial für Etikettierung und Verpackung, umfassend einen Papierträger und eine Glanzbeschichtung, welche auf mindestens einer Seite des Trägers aufgebracht und mit hoher Druckqualität bedruckbar ist;
wobei
die Beschichtung aus einer polymeren Beschichtungszusammensetzung hergestellt ist, welche eine polymerisierbare Basis umfasst, gemischt mit Kaolin, inerten Füllern, Casein und möglichen anderen Additiven; und eine Chromogenzusammensetzung inkorporiert, die sensitiv ist für die Anwendung einer externen Aktivierungszusammensetzung und ausgebildet ist, eine sichtbare Markierung nach der Anwendung der externen Aktivierungszusammensetzung zu erzeugen; wobei die Chromogenzusammensetzung mindestens ein Xanthen-Farbmittel und/oder ein gekapseltes Farbmittel umfasst.

2. Papiermaterial nach Anspruch 1, **dadurch gekennzeichnet, dass** die Chromogenzusammensetzung ausgebildet ist, mit einem in der Aktivierungszusammensetzung enthaltenen Reaktanten oder Lösemittel zu reagieren, um eine Farbgebung in der Beschichtung freizusetzen und die Markierung zu erzeugen.

3. Papiermaterial nach einem der voranstehenden Ansprüche, **dadurch gekennzeichnet, dass** das gekapselte Farbmittel ein vordispergiertes Fettfarbmittel ist.

4. Papiermaterial nach einem der voranstehenden Ansprüche, **dadurch gekennzeichnet, dass** die Chromogenzusammensetzung für eine Chlorderivat-basierte Aktivierungszusammensetzung sensitiv ist.

5. Papiermaterial nach einem der voranstehenden Ansprüche, **dadurch gekennzeichnet, dass** die Chromogenzusammensetzung für eine anorganische Chlorderivatsäuresalze oder organische Chlorderivate enthaltende Aktivierungszusammensetzung sensitiv ist.

6. Papiermaterial nach einem der voranstehenden Ansprüche, **dadurch gekennzeichnet, dass** die Chromogenzusammensetzung für eine lösemittelbasierte Aktivierungszusammensetzung, insbesondere eine polare oder apolare organische lösemittelbasierte Zusammensetzung, sensitiv ist.

7. Authentifizierungs-Kit für Etiketten und/oder Verpackung, umfassend ein beschichtetes Papiermaterial nach einem der voranstehenden Ansprüche und einen Authentifizierungsfilzstift, der ausgebildet ist, die Aktivierungszusammensetzung freizusetzen, um die Chromogenzusammensetzung in der Beschichtung hervorzuheben.

8. Authentifizierungs-Kit nach Anspruch 7, **dadurch gekennzeichnet, dass** die Aktivierungszusammensetzung einen Reaktanten oder ein Lösemittel umfasst, die ausgebildet sind, mit der Chromogenzusammensetzung zu reagieren, um eine Farbgebung in der Beschichtung freizusetzen.

9. Authentifizierungs-Kit nach Anspruch 7 oder 8, **dadurch gekennzeichnet, dass** der Authentifizierungsfilzstift eine Chlorderivat-basierte Aktivierungszusammensetzung enthält.

10. Authentifizierungs-Kit nach Anspruch 9, **dadurch gekennzeichnet, dass** die Aktivierungszusammensetzung anorganische Chlorderivatsäuresalze und/oder organische Chlorderivate enthält.

11. Authentifizierungs-Kit nach einem der Ansprüche 7 bis 10, **dadurch gekennzeichnet, dass** der Authentifizierungsfilzstift eine lösemittelbasierte Aktivierungszusammensetzung, insbesondere eine polare oder apolare organische lösemittelbasierte Zusammensetzung, enthält.

12. Verfahren zur Herstellung eines authentifizierbaren beschichteten Papiermaterials für Etikettierung und Verpackung, umfassend die Schritte: Bereitstellen eines Papierträgers; Herstellen einer polymeren Beschichtungszusammensetzung, umfassend eine polymerisierbare Basis gemischt mit Kaolin, inerten Füllern, Casein und möglichen anderen Additiven; Hinzufügen einer Chromogenzusammensetzung, die sensitiv ist für die Anwendung einer externen Aktivierungszusammensetzung, ausgebildet zum Erzeugen einer sichtbaren Markierung nach der Anwendung der externen Aktivierungszusammensetzung und umfassend ein Xanthen-Farbmittel und/oder ein gekapseltes Farbmittel, zu der Beschichtungszusammensetzung; Aufbringen der die Chromogenzusammensetzung inkorporierenden Beschichtungszusammensetzung auf eine Seite des Trägers, um eine bedruckbare Glanzbeschichtung zu bilden, die eine hohe Druckqualität aufweist und durch Anwenden der externen Aktivierungszusammensetzung authentifizierbar ist.

13. Verfahren nach Anspruch 12, **dadurch gekennzeichnet, dass** die Chromogenzusammensetzung ausgebildet ist, mit einem in der Aktivierungszusammensetzung enthaltenen Reaktanten oder Lösemittel zu reagieren, um eine Farbgebung in der Beschichtung freizusetzen und die Markierung zu erzeugen.

14. Verfahren nach Anspruch 12 oder 13, **dadurch gekennzeichnet, dass** die Chromogenzusammensetzung für eine Chlorderivat-basierte Aktivierungszusammensetzung und/oder eine lösemittelbasierte Aktivierungszusammensetzung, insbesondere eine polare oder apolare organische lösemittelbasierte Zusammensetzung, sensitiv ist.

## Revendications

1. Matériau de papier couché identifiable destiné à l'étiquetage et l'emballage, comprenant un support papier et un couchage brillant appliqué sur au moins une face du support et pouvant être imprimé avec une grande qualité d'impression ;
dans lequel le couchage est composé d'une composition de couchage polymère comprenant une base polymérisable mélangée avec du kaolin, des matières de charge inertes, de la caséine et d'éventuels autres additifs ; et incorporant une composition chromogène sensible à l'application d'une composition activatrice externe et adaptée pour générer un marquage visible après l'application de la composition activatrice externe ; la composition chromogène comprenant au moins un colorant au xanthène et/ou un colorant encapsulé.

2. Matériau de papier selon la revendication 1, **caractérisé en ce que** la composition chromogène est adaptée pour réagir avec un réactif ou un solvant contenu dans la composition activatrice afin de libérer une coloration dans le couchage et générer le marquage.

3. Matériau de papier selon l'une quelconque des revendications précédentes, **caractérisé en ce que** le colorant encapsulé est un colorant gras prédispersé.

4. Matériau de papier selon l'une quelconque des revendications précédentes, **caractérisé en ce que** la composition chromogène est sensible à une composition activatrice à base d'un dérivé chloré.

5. Matériau de papier selon l'une quelconque des revendications précédentes, **caractérisé en ce que** la composition chromogène est sensible à une composition activatrice contenant des sels d'acides organiques chlorés ou des dérivés organiques chlorés.

6. Matériau de papier selon l'une quelconque des revendications précédentes, **caractérisé en ce que** la composition chromogène est sensible à une composition activatrice à base de solvants, en particulier une composition à base de solvants organiques polaires ou apolaires.

7. Kit d'authentification pour étiquettes et/ou emballages, comprenant un matériau de papier couché selon l'une quelconque des revendications précédentes et un marqueur d'authentification adapté pour libérer ladite composition activatrice afin de révéler la composition chromogène se trouvant dans le couchage.

8. Kit d'authentification selon la revendication 7, **caractérisé en ce que** la composition activatrice comprend un réactif ou un solvant adapté pour réagir avec la composition chromogène afin de libérer une coloration dans le couchage.

9. Kit d'authentification selon la revendication 7 ou 8, **caractérisé en ce que** le marqueur d'authentification contient une composition activatrice à base d'un dérivé chloré.

10. Kit d'authentification selon la revendication 9, **caractérisé en ce que** la composition activatrice contient des sels d'acides inorganiques chlorés et/ou des dérivés organiques chlorés.

11. Kit d'authentification selon l'une quelconque des revendications 7 à 10, **caractérisé en ce que** le marqueur d'authentification contient une composition activatrice à base de solvants, en particulier une composition à base de solvants organiques polaire ou apolaires.

12. Procédé de fabrication d'un matériau de papier couché identifiable pour étiquetage et emballage, comprenant les étapes suivantes : la fourniture d'un support papier, la préparation d'une composition de couchage polymère comprenant une base polymérisable mélangée avec du kaolin, des matières de charges inertes, de la caséine et d'éventuels autres additifs ; l'ajout à la composition de couchage d'une composition chromogène sensible à l'application d'une composition activatrice externe adaptée pour générer un marquage visible après l'application de la composition activatrice externe et comprenant un colorant au xanthène et/ou un colorant encapsulé ; l'application de la composition de couchage incorporant la composition chromogène sur une face du support pour former un couchage brillant pouvant être imprimé avec une grande qualité d'impression et identifié en appliquant la composition activatrice externe.

13. Procédé selon la revendication 12, **caractérisé en ce que** la composition chromogène est adaptée pour réagir avec un réactif ou un solvant contenu dans la composition activatrice afin de libérer une coloration dans le couchage et générer ledit marquage.

14. Procédé selon la revendication 12 ou 13, **caractérisé en ce que** la composition chromogène est sensible à une composition activatrice à base d'un dérivé chloré et/ou à une composition activatrice à base de solvants, en particulier une composition à base de solvants organiques polaires ou apolaires
